

## UNITED STATES PATENT OFFICE

2,577,643

## WAX COMPOSITIONS

David W. Young, Roselle, and Arnold J. Morway,  
Rahway, N. J., assignors to Standard Oil De-  
velopment Company, a corporation of Delaware

No Drawing. Application October 11, 1949,  
Serial No. 120,812

6 Claims. (Cl. 106—270)

1

The present invention relates to wax compositions which are suitable for high temperature use and, particularly to waxes which remain stable to heat over extended periods of time.

Several types of waxes may be derived from petroleum oils and in order that no confusion will arise with respect to the types of waxes employed in this invention, a brief description will be given of the method for preparing the waxes used in the present invention.

The term "paraffin" wax is used to define the hard, crystalline wax commonly obtained from petroleum distillates derived from mineral oils of the mixed base or paraffin base type. By the present refining methods, the crude oil is subjected to distillation whereby it is separated into a series of fractions, known as "paraffin distillates." The wax is separated from the paraffin distillate by chilling and filtering or by the use of a solvent as, for example, propane or a ketone, such as methyl ethyl ketone. The wax obtained by either of these methods still contains from 10 to 50% oil and is generally referred to as "slack wax." This slack wax is subjected to a "sweating operation" to remove the oil. The resulting wax usually contains 3 to 6% oil but by proper sweating the oil may be as low as 1 to 3%. This wax known as "crude scale wax" is again sweated to reduce the oil content to less than 0.5% and even as low as 0.05%. This product is known as "refined wax" or "paraffin wax" and is graded according to tensile strength, melting point, oil content, hardness, etc.

It has been suggested in the prior art that for some purposes it is advantageous to add certain metal salts, particularly the metal salts of organic fatty acids to paraffin waxes. Various investigators have found that the addition of metal salts of the character referred to have utility for improving the tensile strength and melting point of the wax. There appear to be several theories as to the operation of such metal salts in conjunction with the soaps. One such theory is that the addition of salts of low molecular weight acids to soaps of relatively high molecular weight results in the formation of a complex with superior grease thickening effect and of improved stability.

Suggestions in the prior art have included the use of the salts of saturated fatty acids, such as stearic and oleic acids. However, these salts are difficult to solvate, temperatures of about 400° F. being required.

According to the present invention, the salts of

2

certain acids, particularly the salts of heterocyclic acids, such as furoic acid, are highly useful as ingredients of waxes. Furoic acid, for example, may be readily derived from furfural which is abundantly available at low prices at this time. Thiofuroic acid may be used. Other related compositions appear also to be similarly useful, for example, alkyl furoic acid, thiophene carboxylic acid, etc. These compounds all have five membered furan-type rings and are of low molecular weight.

The use of the salts of acids of the type set forth above, such as furoic acid, is not to be confused with the use of related esters which have entirely different purposes. Thus, it has been suggested in the prior art, Zimmer et al. Patent No. 2,113,754, dated April 12, 1938, that certain furoic acid esters are useful as oiliness agents in various lubricating compositions. This reference suggests that such esters may be used either in lubricating oil or lubricating greases. The esters, however, are entirely different from the salts employed in the present instance and their function is not related in any way to the function of the furoic acid salts and the equivalent compositions of low molecular weight heterocyclic acids.

U. S. Patent No. 2,388,166 recites the use of lithium stearate and other lithium salts of mono- or polybasic aliphatic carboxylic acids containing at least eight carbon atoms to increase the melting point of the wax. However, these materials as shown below do not have the beneficial properties of the addition agents of the present invention.

In the present case, the low molecular weight salts are added to the wax for the purpose, as indicated above, of improving high temperature stability of the wax and also to increase its tensile strength.

In general, the metallic element of the salts may be any of the alkali or alkaline earth metals. Sodium and lithium are preferred of the alkali metals and calcium is the preferred alkaline earth metal partly because of its low cost. Salts of potassium, strontium, magnesium and barium may be used, however, as well as the soaps of any of these metals and mixtures of salts and/or soaps of any or all of the alkali and alkaline earth metals also are contemplated. The relative proportions of the salts added may vary from 1 to 5%.

The following table illustrates the improved tensile strength and heat stability of the wax

composition of the present invention containing lithium salt of furoic acid in comparison with a wax containing lithium stearate:

TABLE  
*Lithium salts in paraffin wax*

| Name of Compound                            | Per Cent Additive | M. Pt.,<br>ASTM<br>D127-30 | Penetration,<br>ASTM D5-25,<br>77° F. | Tensile,<br>Lbs./34" | Heat <sup>1</sup><br>Stability |
|---------------------------------------------|-------------------|----------------------------|---------------------------------------|----------------------|--------------------------------|
| Paraffin Wax                                | 0                 | 130                        | 12                                    | 61                   | fair.                          |
| +1% Li stearate                             | 1                 | 138                        | 11                                    | 73                   | Do.                            |
| +3% Li stearate                             | 3                 | 144                        | 11                                    | 94                   | Do.                            |
| Paraffin Wax +1% Li salt<br>of furoic acid. | 1                 | 135                        | 11                                    | 74                   | good.                          |
| Paraffin Wax +3% Li salt<br>of furoic acid. | 3                 | 144                        | 11                                    | 90                   | Do.                            |

<sup>1</sup> A 50 gram sample of each sample was placed in a Pyrex beaker, covered with a watch glass and held at 70° C. for eleven days in a circulating air oven and the samples tested for odor daily. At the end of the test the samples were evaluated for taste as well as for odor. The results were labeled according to the following schedule:

Excellent—No taste and odor.

Good—An odor but not objectionable; no taste.

Fair—Slightly objectionable odor and taste.

Poor—Objectionable odor and taste.

The above data indicate that the tensile strength of the wax composition containing lithium salt of furoic acid is equally as good as that of a wax containing lithium stearate while the heat stability is remarkably increased.

In the data given above, the lithium salt of furoic acid was used as the addition agent, although the invention can be carried out with other alkali and alkaline earth salts.

The nature of the present invention having been fully set forth and specific examples of the same given, what is claimed as new and useful and desired to be secured by Letters Patent is:

1. A wax composition consisting essentially of refined paraffin wax and 1 to 5% of a metal salt chosen from the class consisting of alkali metal and alkali earth salts of a heterocyclic carboxylic acid, said heterocyclic acid being a low molecular weight acid having a five-membered furan-type ring.

2. A wax composition consisting essentially of

refined paraffin wax combined with 1 to 5% of an alkali metal salt of a heterocyclic carboxylic acid, said heterocyclic acid being a low molecular

weight acid having a five-membered furan-type ring.

3. A wax composition according to claim 2 wherein the metal salt is the lithium salt.

4. Composition as in claim 1 wherein said metal salt is an alkaline earth metal.

5. A wax composition suitable for high temperature service consisting essentially of refined paraffin wax and 3% of an alkali metal salt of furoic acid.

6. Composition according to claim 5 wherein said metal salt is the lithium salt.

DAVID W. YOUNG.  
ARNOLD J. MORWAY.

#### REFERENCES CITED

The following references are of record in the file of this patent:

#### UNITED STATES PATENTS

| Number    | Name  | Date         |
|-----------|-------|--------------|
| 2,284,065 | Myers | May 26, 1942 |